

## UNITED STATES PATENT OFFICE

ALBERT W. DROBILE, OF CYNWYD, PENNSYLVANIA

## PILE FABRICS AND METHOD OF MAKING THE SAME

No Drawing.

Application filed April 8, 1929. Serial No. 353,660.

My invention is an improved pile fabric having the loops of the pile united to the backing fabric by the solidified pliable composition resulting from the coagulation in situ on the backing of an aqueous colloidal dispersion of previously uncoagulated rubber which, by reason of its affinity for the fibres and the capillary actions thereof, intimately permeates the fibres of the backing 5 and pile and forms a bond between them quite different from and superior to the effect of coating pile fabrics with organic solutions of rubber and other non-aqueous substances heretofore proposed for use in 10 coating pile fabrics. In the preferred embodiment of my invention, the aqueous dispersion of rubber contains vulcanizing substances preferably in colloidal form, which are carried into the pores of the fibres and facilitate the coagulation or vulcanization 15 of the rubber in such pores as well as in the interstices between the fibres so that the pile is embedded in a substantially continuous film which not only firmly anchors the pile 20 and reenforces the backing but tends to render the fabric impervious to moisture without detracting from the appearance or feel of the fabric or of the pile thereof. The composition is insoluble in water after solidification, and may be colored or embossed 25 to give desired effects independently of or in conjunction with pile decoration resulting from printing, cutting, singeing, acid treatment or the like.

30 The aqueous dispersions of rubber which I have found most suitable for use on pile fabrics contain vulcanizing agents, such as colloidal sulphur, zinc oxide and an accelerator, and these constituents may either be 35 retained inert in the aqueous rubber until after coating is completed, or they may be permitted to vulcanize, without coagulating, the rubber before coating the fabric.

When a prevulcanized coating is used, the 40 film is "set" by the evaporation of the watery constituent of the coating, which is preferably done by the application of a moderate drying heat or a vacuum, which causes the coagulation of the rubber content 45 into an impervious film intimately permeat-

ing the backing and a desired portion of the pile. When an unvulcanized coating containing vulcanizers is used, the coated fabric is preferably subjected to a vulcanizing heat, which both vulcanizes and coagulates the 55 coating.

55 My improvements are particularly applicable to the treatment of pile fabrics woven on the double plush principle, which may be woven with relatively few picks or weft threads over which the pile warps are looped. Such loosely woven fabrics when split apart are ordinarily unfitted for usage 60 because the pile fibres are easily shed from the backing and the backing lacks firmness or body. Moreover certain fibres have too much resilience to be satisfactorily looped and held firmly in even a tightly woven 65 backing without being secured by backing picks or being floated in the backing. By 70 the utilization of my improvements, the pile is firmly embedded regardless of the looseness of the backing or the resiliency of the pile fibres, and the loose backing is filled or weighted by the film deposited in the 75 pores of the fibres thereof so as to give the feel and wear of a closely woven backing, and the pile may be closely cut to form a 80 very short nap without causing shedding, despite the fact that each pile is looped over but a single pick.

85 By the practice of my invention, a pile fabric may be inexpensively woven with a dense face of animal fibres, such as mohair, looped around each pick or weft thread 85 without floating the pile warps in the backing or anchoring them by locking picks. Such fabrics, particularly when the piles are cut short or the wefts are lightly beaten up are unsuitable for the use to which the 90 fabrics are to be put but are rendered suitable for such use and given greater durability than usual pile fabrics by uniting the pile loops and backing threads in a continuous film resulting from coating on the back of the fabric an aqueous dispersion of rubber containing a vulcanizer and accelerator which is drawn into intimate relation with the fibres by the capillary action thereof upon the 95 coating.

The coating composition is preferably gradually fed to the backing fabric adjacent to a knife or scraper by which it is evenly spread over the surface, but may be applied in any suitable manner, and either after or before the pile has been split to separate the double backings. After coating, the fabric is preferably immediately subjected to a drying, coagulating or vulcanizing heat depending upon the characteristics of the particular aqueous dispersion of rubber used. After the coating has set, the fabrics may be dyed and finished without the difficulties heretofore experienced from the bleeding of relatively large volumes of dye from previously dyed backing thread into the final face-dying bath of dye, and the usual bichromate treatment of the backing after dying to prevent such bleeding may be eliminated.

The fabrics produced may be decorated by cutting, singeing, embossing or acid treatment in any usual way.

Having described my invention, I claim:

25 1. An improved pile fabric having loops of the pile containing animal fibre united to the backing fabric by a solidified pliable composition resulting from the coagulation in situ on the backing of an aqueous dispersion of rubber permeating the interstices of said fabric.

30 2. An improved pile fabric having loops of the pile containing animal fibre united to the backing fabric of predyed yarn by a solidified pliable composition resulting from the coagulation in situ on the backing of an aqueous colloidal dispersion of previously uncoagulated rubber and a vulcanizer.

35 3. An improved pile fabric comprising a backing of predyed yarn containing resilient pile warps containing animal fibre and too loosely bound by said backing to alone securely hold said warp threads for the use to which the fabric is to be put and a film capillary permeating said backing and pile warp and consisting of a previously uncoagulated aqueous dispersion of rubber and said pile containing dye uncontaminated by bleeding from said predyed 40 yarn.

45 4. The method of making pile fabric which comprises weaving a loose textile backing of predyed threads with pile warps containing animal fibre loosely looped over the picks of said backing and permeating said backing and pile loops by capillary action with an aqueous dispersion of rubber applied to said backing opposite the pile.

50 5. The method of making pile fabric which comprises weaving a loose textile backing with resilient pile warps containing animal fibre loosely looped over wefts of said backing and permeating said backing and pile loops by capillary action with an aqueous dispersion of rubber containing a vul-

canizing agent and vulcanizing said rubber in situ.

6. The method of making pile fabric which comprises weaving a loose textile backing of predyed yarn with resilient pile warps containing animal fibre and loosely looped therein and permeating said backing and pile loops by capillary action with an aqueous dispersion of rubber containing an emulsifying agent and an accelerator.

7. The method of making pile fabric which comprises weaving a loose textile backing with pile warps containing animal fibre loosely looped therein, permeating said backing and pile loops by capillary action with an aqueous dispersion of rubber, coagulating said rubber by heat, and dying and finished the coated fabric.

8. The method of making pile fabric which comprises weaving a loose textile backing from previously dyed backing threads and looping pile warps containing animal fibre loosely over wefts of said backing, permeating said backing and pile loops by capillary action with an aqueous dispersion of rubber containing a vulcanizer, coagulating said rubber, and face-dying said fabric.

In testimony whereof I have hereunto set my hand this sixth day of April, 1929.

ALBERT W. DROBILE.

70

75

80

85

90

95

100

105

110

115

120

125

130